

## UNITED STATES PATENT OFFICE

2,606,325

AGE AND STAIN-RESISTING ARTICLE OF  
PLASTICIZED POLYVINYL CHLORIDE

Carl A. Nielson, Takoma Park, and Fred Leonard, Silver Spring, Md., and Irving Cort, Washington, D. C., assignors to the United States of America as represented by the Secretary of the Army

No Drawing. Application August 1, 1949,  
Serial No. 108,046

2 Claims. (Cl. 3-1)

(Granted under the act of March 3, 1883, as  
amended April 30, 1928; 370 O. G. 757)

1

The invention described herein may be manufactured and used by or for the Government for governmental purposes, without payment to us of any royalty thereon.

There has been made in recent times marked progress in the production of gloves or coverings for prosthetic hands, which gloves simulate in high fidelity the appearance and texture of a natural hand, thereby rendering inconspicuous to an observer the deformity resulting from an amputation and use of an artificial or prosthetic hand.

Such gloves essentially duplicating the appearance of a natural hand in color and surface markings are being obtained by molding or casting a vinyl chloride polymer and plasticizer therefor in a seamless, one-piece metal (nickel) mold and heating the cast resin while in the mold to an elevated temperature to effect solution of the swelled or gelled resin in the plasticizer and develop the maximum tensile strength and tear resistance. The glove then is removed from the mold and pigmented interiorly to match the color of a natural mating hand.

In the course of use, the glove comes into contact with many different varieties of materials which tend to stain or to discolor the glove in a permanent manner, such staining detracting from the appearance and wearing qualities of the glove. It has been found in practice that a plasticized polyvinyl chloride glove is stained irreversibly by a wide variety of materials. This staining is due to the high solvent power of the plasticizer in the composition towards various oil-soluble dyes used in shoe polish, ball-point ink, and many other materials.

Not only in connection with the production of gloves but in connection with many other applications of vinyl resins, continued advances have been made in the technology of vinyl resins through modifications, combinations and development of improved plasticizers, pigments and processing. Through these advances, many uses for such resins have been found and exploited, such as shower curtains, raincoats, umbrellas, furniture upholstery, and flooring material. Military uses for the resins include gun covers, tent windows, coated fabrics, maps, and vinyl coatings on metals. The use of the vinyl resins in the aforesaid "cosmetic" gloves for amputees, both civilian and military, is a very recent use of such resins.

While many advantages may be listed in favor of plasticized polyvinyl chloride-type resins, there are several disadvantages which arise principally from the inability of the stocks to resist soilage. Incorporation of the above-indicated enhanced

properties in polyvinyl chloride stocks would undoubtedly result in increased application and utility.

In connection with the use of plasticized vinyl chloride polymers in cosmetic gloves the problem of irreversible soilage is of extreme importance. For example, gloves worn by amputees over an extended period of time tend to become somewhat dark and glossy before the wearing life of the gloves has become exhausted; and rubbing against newsprint, clothing, or the like, which is inevitable during wearing of the gloves, is found to have a tendency to produce stains which cannot be removed readily by soap and water or the usual solvents without producing undesirable effects.

The present invention provides a process for preventing the deleterious effects of irreversible soilage and aging on plasticized polyvinyl chloride stocks; and while not limited to cosmetic gloves, the invention is of especial applicability thereto, as it affords full protection without obliterating or obscuring any of the fine surface details or natural appearance which characterize such gloves produced from plasticized polyvinyl chloride.

In accordance with the present invention, it has been found that coating the plasticized polyvinyl chloride stocks with the unplasticized copolymer of ethyl acrylate and acrylonitrile (90 parts to 10 parts respectively) of high molecular weight, an excellent adhesion of the copolymer as a coating film to the plasticized polyvinyl chloride stocks can be obtained, and the resulting coated stocks remain free from the objectionable disadvantages that are found to be inherent in the polymerized polyvinyl chloride. For depositing a flexible film of the 90-10 copolymer of ethyl acrylate and acrylonitrile, the flexible film being free from plasticizing constituents for the said polymer, it is merely necessary to spray a latex dispersion or solution of the copolymer on the plasticized polyvinyl chloride sheet or shape and allow it to dry. An oven may be used to hasten the drying time.

The unplasticized copolymer of ethyl acrylate and acrylonitrile may be prepared by polymerizing these materials together at from about 15° C. to about 20° C. in a sealed container using potassium persulphate as catalyst, and in the presence of a reducing agent, for example sodium hyposulphite, about 0.5 per cent by weight of resins being the catalyst and sodium hyposulphite. An aqueous dispersion of the resulting copolymer is obtained as an aqueous latex emulsion.

More specifically, the emulsion may be prepared

from the following constituents and in accordance with the following procedure, such illustrating the preferred constituents and operational procedures for producing the desired coating:

| Ingredients:                         | Parts by weight |
|--------------------------------------|-----------------|
| Ethyl acrylate                       | 90              |
| Acrylonitrile                        | 10              |
| Potassium persulphate (catalyst)     | 0.5             |
| Sodium hyposulphite (reducing agent) | 0.5             |
| Santomerse D (100 parts of 1%)       | 1               |
| Water                                | 99              |

The "Santomerse D" employed in the foregoing illustrative composition is one of the series of santomerse manufactured by the Monsanto Chemical Company. The santomerse are salts of a homologous series of substituted aromatic sulphonic acids, used as wetting, spreading, penetrating, and emulsifying agents.

#### *Production of the emulsion*

To a solution of the Santomerse D in water contained in a bottle there were added the ethyl acrylate and acrylonitrile. The mixture was placed on a shaking machine and agitated until the emulsion appeared homogeneous, this requiring about five minutes. The persulphate and thiosulphate were added, the bottle sealed and placed in a polymerization bath and rotated end over end at 20° C. Approximately eight hours is sufficient to obtain complete polymerization. The emulsion of the polymerized monomers thus formed is applied to the plasticized polyvinyl chloride base. The emulsion may be applied by spraying, brushing, or the plasticized polyvinyl chloride base may also be dip-coated.

It is found, surprisingly enough, that the emulsion when dried to form the coating, in no way impairs the desired qualities of the plasticized polyvinyl chloride sheet or base, and actually renders the base highly resistant to irreversible soilage and aging. For example, an uncoated sheet and a coated sheet were marked both with a ball point pen and rubbed with newsprint. The specimens then were washed with soap and water or water-alcohol mixtures, and the resulting stains were easily removed from the coated sheet, whereas the uncoated sheet resisted removal. A similar result was obtained with a coated plasticized polyvinyl chloride cosmetic glove, as compared with an uncoated glove.

As applied, the coating is a transparent, elastic film, tightly adherent to the base. Application of the technique of this invention to a molded cosmetic glove made of plasticized polyvinyl chloride shows that the deposition of the flexible ethyl acrylate-acrylonitrile copolymer film causes no impairment of the convincing detail inherent in the original unsprayed glove.

The coating is, as has been pointed out above, an emulsion dispersed or solution dispersed copolymer of ethyl acrylate and acrylonitrile. As prepared, the material has a tensile strength of approximately 800-900 pounds per square inch, an elongation of approximately 600-700% and a 100% modulus of 70 pounds per square inch, and good recovery. The low modulus and high elongation compared to the plasticized polyvinyl chlo-

ride glove makes it possible to flex the glove repeatedly without causing the coating to crack and peel.

The adherent bond between the plasticized polyvinyl chloride base and the coating is due probably to hydrogen bonding between the plasticizer in the polyvinyl chloride resin and the rather active tertiary hydrogen alpha to the negative cyanide or carbonyl group in the copolymer. The adhesive bond is higher in magnitude than the breaking strength of the copolymer.

While the use of the 90-10 copolymer of ethyl acrylate and acrylonitrile is preferred as the protective coating in accordance with this invention, the invention is not limited to the use of such copolymer, as copolymers of varying compositions may be used, and similar results may be obtained with latices of polyethyl acrylate and other esters of acrylic acid, such as methyl acrylate, butyl acrylate and other higher alkyl acrylates and copolymers thereof.

Having thus described our invention, what we claim as new and wish to secure by Letters Patent is:

1. As a new article of manufacture, a freely flexible base composed of plasticized polyvinyl chloride having bonded thereto a continuous and permanent coating film composed essentially of an unplasticized copolymer of ethyl acrylate and acrylonitrile containing approximately 90 parts by weight of ethyl acrylate and 10 parts by weight of acrylonitrile, the film having a flexibility substantially greater than that of the base and characterized by high resistance to irreversible soilage and aging.

2. As a new article of manufacture, a cosmetic glove for covering an artificial hand and duplicating in high fidelity all surface characteristics of a natural hand the said glove being composed of a freely flexible plasticized vinyl chloride polymer base and a continuous transparent coating film covering permanently coating the base and composed of the copolymers of ethyl acrylate and acrylonitrile containing approximately 90 parts by weight of ethyl acrylate and approximately 10 parts by weight of acrylonitrile, the said coating being continuously adherent to the base and having a flexibility substantially greater than that of the base and characterized by high resistance to irreversible soilage and aging, thereby protecting the plasticized vinyl chloride polymer base against deterioration by aging and irreversible staining.

CARL A. NIELSON.  
FRED LEONARD.  
IRVING CORT.

#### REFERENCES CITED

The following references are of record in the file of this patent:

#### UNITED STATES PATENTS

| Number    | Name          | Date          |
|-----------|---------------|---------------|
| 2,060,342 | Palicki       | Nov. 10, 1936 |
| 2,332,461 | Muskat et al. | Oct. 19, 1943 |
| 2,453,604 | Tenenbaum     | Nov. 9, 1948  |
| 2,473,723 | Nelson        | June 21, 1949 |
| 2,491,097 | Feagin        | Dec. 13, 1949 |
| 2,491,102 | Frowde        | Dec. 13, 1949 |